

Patented June 11, 1929.

1,717,316

# UNITED STATES PATENT OFFICE.

GEORGES HEBERLEIN, OF WATTWIL, SWITZERLAND, ASSIGNOR TO HEBERLEIN PATENT CORPORATION, OF NEW YORK, N. Y., A CORPORATION OF NEW YORK.

## TREATMENT OF VEGETABLE FIBROUS MATERIAL TO PRODUCE WOOLLIKE EFFECTS.

No Drawing. Application filed October 30, 1926, Serial No. 145,381, and in Germany August 19, 1926.

This invention relates to the treatment of vegetable fibrous material and resulting product, and more particularly to the production of wool-like effects on vegetable fibrous material. The invention is applicable to the treatment of vegetable fibrous material such for example as cotton fibres, whether in loose form or in yarns or fabrics.

It is known from various prior patents such as some of my own prior patents, that vegetable fabrics experience a contraction in consequence of treatment with reagents that have a swelling action on the vegetable fibres if the reaction is allowed to take place without hindrance in a loose state of the goods, i. e., without a counteracting tension. In consequence of the contraction of the fibres during the treatment the fabric becomes more dense and is given a certain wool-like character, i. e., like fine thin woolen fabric.

The object of the present invention is to obtain a wool-like effect in a simple and less expensive manner than heretofore obtainable.

It has been discovered in accordance with this invention that augmented and more pronounced wool effects are obtained if caustic alkali solutions of previous known mercerizing strengths and preferably caustic soda are caused to act upon the raw vegetable fibres, i. e., fibres which still have the natural incrustations or coatings adhering to them and while the material is allowed to lay loose to attain full shrinkage due to the swelling agent, and if the usual bleaching by alkali boiling is entirely excluded; that is to say, if the fibres are subjected to any alkali treatment before the swelling reagent acts, such alkali treatment shall be simply a gentle bleaching, preferably a cold bleaching, as distinguished from the customary alkali boiling; and on the other hand, if there is to be no preliminary alkali treatment before the swelling reagent is applied, but there is to be an alkali treatment or bleaching after the swelling agent acts, then again such subsequent alkali treatment must be merely a gentle bleaching, preferably a cold bleaching, as distinguished from a bleaching by alkali boiling. It is essential that alkali boiling be excluded, and that if there is a cleansing of the vegetable fibres before or after the swelling treatments it should be merely a careful cleansing without alkali boiling. It is important to keep the material in a loose state throughout the process starting with the

swelling agent, so as not to prevent or materially impair or reduce the fully shrunk effect. Even in drying, the material should only be stretched enough to remove folds or creases.

An expedient method of procedure is, for example, to subject the raw fabrics to a weak preliminary cleansing to remove the dressing, say for example with dilute acid or diastase or similar ferments, and therupon to introduce the fabrics into the caustic solution. After completion of the swelling reaction and removal of the surplus swelling agent, there follows the bleaching of the goods, provided such bleaching is desired. In this one should proceed very gently, and if bleaching is desired, it is best to adopt the means of cold bleaching and to avoid all alkaline boiling. The cold bleaching may be carried out by cold or only slightly heated alkaline hypochlorite solutions; cold hydrogen peroxide or sodium peroxide baths are also suitable.

As an alternative procedure, one may first subject the raw fabric to a gentle bleaching and then cause the caustic to act upon it.

The swelling must be carried out in such a manner that a tensing of the fabric is obviated. This may be effected by carefully laying the fabric into vats, or else use may be made of a machine for continuous treatment of the fabric. Such a machine should provide suitable means for subjecting the fabric in an untensioned or loose state to the swelling agents as the fabric is moved along, and with means for squeezing out the excess swelling agent and for thereafter supporting the fabric in loose state, such as fanwise or in folds, and carrying it along, so that the contraction of the fabric is permitted to work itself out completely due to the action of the swelling agent thereon, after which the fabric may be passed through suitable washing means and allowed to dry, care being taken that the considerably shrunk fabrics shall not be stretched or tensioned to an extent to substantially reduce or counteract the shrinkage obtained.

After the termination of the treatment the fabrics may be dyed and printed in any desired manner.

As a concrete example of the manner in which the process may be carried out on cotton fabrics, I give the following: The grey goods are desized, that is, well washed out

but not bleached or boiled; after which the goods are ready to be treated by the swelling agent. This may be done preferably by the use of some suitable machine by means of which the goods is impregnated with the swelling reagent which in this case is caustic soda, of a strength of approximately 30° Bé. at a temperature of approximately 15° C., the goods being subjected to this reagent 10 while in loose state as stated, and after such action by the reagent the goods are not immediately washed out but are left in loose condition for say 10 or 20 minutes under the influence of the retained swelling agent, so 15 that the goods have time to shrink thoroughly. In some instances the goods may be impregnated twice before they are left to lay loose as stated. After the shrinkage has taken place the goods may be washed, 20 soured, again washed and then dried without tension. That is to say, in drying the goods should only be stretched sufficiently to take out the folds but not sufficiently to materially reduce or counteract the shrinkage obtained.

The result is a wool-like finish of the general character of that described and claimed in my United States Patent No. 1,392,264, granted September 27, 1921, obtainable in a 30 less expensive and more ready manner.

The process may be applied to all kinds of fabrics, to woven and knit goods, embroidery, as well as all other vegetable fibrous products that have a surface. This improvement is 35 likewise applicable to products made of mixtures of vegetable fibres with animal fibres as well as with artificial fibrous materials.

In accordance with this invention the well-known crepon effects can also be attained 40 with special softness by this means, that the swelling agents are caused to act locally upon the raw or only slightly cleansed fabrics. At the spots where the swelling agent acts, the fibre contracts and a soft wool-like 45 effect is formed, while the unchanged spots of the fabric bulge out like blisters or swollen parts. The application of the swelling agents may be effected by direct imprinting, or one may proceed by means of resist printing and subsequent impregnation. In the 50 case of the resist printing, dyes may at the same time, in well-known fashion, be locally incorporated in the fibre, or fabrics that have been previously dyed may be locally dis- 55 charged by means of the resist so as to be white or colored. By means of subsequent dyeing of the crepon effects manifold dye effects are obtained.

While I have described my invention with 60 particularity in accordance with one preferred method of carrying out the same, it will be obvious to those skilled in the art, after understanding my invention, that various modifications and changes may be made 65 therein, and I aim in the appended claims to

cover all such changes and modifications as come within the spirit and scope of the invention.

Having thus described my invention, what I claim as new and desire to secure by Letters 70 Patent, is:

1. Process of producing wool-like effects on vegetable fibrous material i. e. effects like fine thin woolen fabric, which comprises taking vegetable fibrous material which has 75 not been subjected to an alkali boiling, and treating such material in loose state with caustic alkali which will produce a swelling action on the vegetable fibres, maintaining the material in loose state and under the influence of said caustic alkali until said material has been swollen by said caustic alkali and substantially fully shrunk, then treating the material so as to eliminate further effect 80 of the caustic alkali, and drying the material 85 without such stretching as would substantially reduce the attained shrinkage and without subjecting the material to an alkali boiling.

2. Process of producing wool-like effects 90 on fabrics containing vegetable fibres i. e., effects like fine thin woolen fabric, which comprises taking such fabric which has not been subjected to an alkali boiling and treating such fabric in loose state with caustic alkali 95 of sufficient strength to produce a substantial swelling action on the vegetable fibres, maintaining the fabric in loose state and under the influence of said caustic for several minutes and until said fibres have been swollen 100 by said caustic and substantially fully shrunk, then treating the fabric so as to eliminate the further effect by said caustic, and drying the fabric without such stretching as would substantially reduce the attained 105 shrinkage and without subjecting the fabric to an alkali boiling.

3. Process of producing wool-like effects on fabric containing cotton fibres, i. e., effects like fine thin woolen fabric, which comprises taking for treatment such fabrics in the grey or raw state, treating the raw fabric in loose state with caustic soda of sufficient strength to produce a substantial swelling action on the cotton fibres, maintaining the 110 fabric in loose state and under the influence of said caustic for several minutes and until said cotton fibres have been swollen by said caustic and substantially fully shrunk, and then washing and drying the fabric without 115 such stretching as would substantially reduce the attained shrinkage, and without subjecting the fabric to an alkali boiling.

4. Wool-like effect fabrics, i. e., like fine thin woolen fabric, made in accordance with 120 the process of claim 2.

In testimony whereof I have signed my name to this specification.

GEORGES HEBERLEIN,